

## UNITED STATES PATENT OFFICE

2,053,046

## PENETRATING OIL

Anderson W. Ralston, William O. Pool, and James Harwood, Chicago, Ill., assignors to Armour and Company, Chicago, Ill., a corporation of Illinois

No Drawing. Application August 27, 1935,  
Serial No. 38,137

6 Claims. (Cl. 87—9)

This invention relates to penetrating oils and to processes of using the same and it comprises a penetrating oil in which the predominantly active constituent is an aliphatic nitrile containing six or more carbon atoms, and it further comprises processes of loosening adherent deposits on metallic surfaces by the application thereto of such penetrating oils.

There is a demand in the arts for liquids which have the property of penetrating readily between metal surfaces in close contact, such as the leaves of springs, hinges, bolts, and the like. The difficulties in loosening bolts which have "rusted" are well known. This layer or film of rust is so tenacious that very often it binds the adjacent metal surfaces so tightly that it is difficult, if not impossible, to loosen the bolt by the mere application of mechanical loosening devices such as a wrench. Frequently door hinges develop "squeakiness", due at least in part to the formation of thin films of rust between the moving parts of the hinge. And it is commonly necessary to "lubricate" the springs of an automobile by the application thereto of so-called penetrating oils.

All of the oils which have been used for this purpose must have high penetrability. This means that the surface tension and viscosity of the oil should be somewhat lower than that of an ordinary lubricant used on rotating parts. A penetrating oil is one which has the ability to form a lubricating film between closely contacted metal parts. This is to be distinguished from oiliness in oil. Oiliness is the ability of the film to adhere to the metal once the film is formed.

Penetration is not possessed to any decided degree by ordinary lubricating oils and in order to improve this characteristic various materials have hitherto been added to them. Oil of citronella, various other essential oils, ethers, and esters have been used. Many of these addition agents are unsatisfactory. Most of them are rather fugitive substances and they readily oxidize and decompose.

We have now discovered that a class of chemical compounds known as higher fatty acid nitriles have excellent properties of penetration and lubrication when applied to metallic surfaces. We find that these nitriles will readily penetrate rusted surfaces between bolts and hinges, for example, where ordinary lubricants fail to function. We are not prepared to state exactly what happens when the penetrating oils of our invention are applied to rusted surfaces but we do believe that they function chemically in some way to loosen the bond between the particles of rust

and the metal surface to which rust adheres tenaciously. Although there are many mineral lubricating oils of very low viscosity having some penetrability, many of these oils, after penetration, are not particularly effective for the purpose of loosening rusted surfaces. There is no reason for believing an ordinary mineral hydrocarbon would have any particular chemical reaction with the rust. On the other hand the nitriles of the present invention are rather active compounds chemically and, although they may appear to be substantially inert with respect to a rusted surface, we believe that they do have some definite chemical reaction with the surface of the rusted particles so that any tenacious bond between the metal and its coating of rust is loosened. In many respects this would seem to be analogous to the pickling and cleaning of metals wherein obscure chemical reactions do occur.

We have further discovered that these aliphatic nitriles are excellent carbon removers. They can, for instance, be sprayed on the layer of carbon deposit on the surface of the cylinder of an internal combustion engine, or the cylinders can be flushed with them. When the engine is then started up, the carbon layer is loosened by the nitrile and blown out. An ordinary mineral oil, regardless of its viscosity, will not lessen such carbon deposits. Accordingly, we believe that the action of our materials must be something more than a mere mechanical penetration or working in between metallic surfaces or carbon deposits on a cylinder wall.

In its broad aspects, then, our invention relates to the use of the higher fatty acid nitriles, that is, nitriles containing at least six carbon atoms, for the purpose of loosening adherent deposits on metallic surfaces, the deposits being of the nature of rust or carbon.

There are many nitriles coming within the scope of our invention. All of them are free flowing liquids of low viscosity. These nitriles are customarily made from fatty acids by reacting the fatty acids with ammonia in the presence of a dehydrating catalyst. Thus stearonitrile and palmitonitrile are nitriles corresponding to stearic and palmitic acids. Nitriles corresponding to the other higher fatty acids can be prepared in like manner and used in our invention. For example, we can use nitriles prepared from capric, caprylic, lauric, myristic and the unsaturated fatty acids such as oleic and linoleic.

We can also use products obtained by pyrolytically cracking higher fatty acid nitriles such as stearo- and palmitonitrile. These cracked prod-

ucts are mostly lower molecular weight fatty acid nitriles, both saturated and unsaturated, and which boil from 40° C. to as high as 360° C. In many instances the cracked nitriles are associated with quantities of hydrocarbons which are also products of the cracking reaction. Methods of preparing these cracked nitriles are described in the copending applications Serial Numbers 9,660 and 11,348 filed by us, now Patents 2,033,536 and 2,033,537. These methods involve heating nitriles, such as stearonitrile, at a temperature of about 550° C. with or without a catalyst and either at ordinary or elevated pressures.

As stated above, in broad aspects our invention 15 comprises the use of these nitrile materials for the purpose stated. For example, we prepare a mixture containing about equal parts of palmito and stearonitrile all of which has a boiling point somewhat higher than 340° C. This mixture penetrates between metallic surfaces readily and quickly loosens rusted bolts, hinges, and the like. Another mixture which we can use is that composed of the nitriles from lard fatty acids. In 20 making this mixture we convert the lard fatty acids to their corresponding nitriles in ways well known. The nitrile mixture obtained will contain nitriles mostly corresponding to palmitic and oleic acid. Its boiling point range is about 320° C. to 355° C.

Similarly a mixture of nitriles consisting of the cracked reaction product resulting from the cracking of stearo and palmito nitriles will give 25 excellent results as a penetrating oil. The exact composition of this mixture is not known but we do know that it contains nitriles having from seven to twelve carbon atoms. Such nitrile mixtures are described in the copending applications referred to above.

We have also discovered that these nitriles can 30 be added to and dissolved in lubricating oils with advantage. Thus, when we add one part of the nitrile by volume to nine parts of the lubricating oil by volume, the penetrability of the lubricating oil is markedly increased. Such an oil used 35 on rusty bolts works very well but in the absence of the nitriles the lubricating oil has no loosening effect. In a similar manner we can improve the penetrability of all of the common mineral oils used for lubricating purposes. These oils can 40 range in viscosity from a number 10 SAE to a 30 or 40 SAE but we ordinarily do not treat lubricating oils of higher viscosity than this since in most instances such oils are too viscous and it is difficult to increase their penetrability characteristics 45 except at the expense of adding very large

quantities of nitriles. The amount of nitrile or mixtures thereof which we dissolve in the lubricating oil is not at all critical. In most instances it amounts to about 5 to 20 percent of the mineral oil.

Any of the above-described nitriles, or mixtures thereof, or the cracked nitriles, can be compounded with mineral lubricating oils to give oils of superior penetrability and "loosening" effect.

One very advantageous mixture will contain 10 about 80 parts by volume of a number 20 SAE lubricating oil, about 10 parts by volume of stearonitrile and about 10 parts by volume of palmito nitrile. These quantities can be varied over wide limits, so that the mineral oil contains 15 from 5 to 20 percent of stearonitrile alone, or admixtures thereof with palmitonitrile. Similarly we can replace the stearo and palmitonitrile with the cracked nitriles described above. Thus our oil can contain from 5 to 20 percent of 20 cracked nitriles having from six to twelve carbon atoms.

As stated, we do not ordinarily incorporate our nitriles in lubricating greases. We can, however, improve the lubricating properties of 25 greases as regards their penetrability by adding our nitriles thereto and we do not intend the appended claims to be limited to highly fluid products. We can, for example, add from 5 to 30 percent of the above nitriles, or mixtures thereof, to 30 a mineral lubricating grease. This will increase the penetrability of the grease and improve its lubricant film-forming properties considerably. Such uses are indicated in greases for gear lubrication, spring shackles and the like.

Having thus described our invention what we claim is:

1. As a new composition of matter, a mixture of a mineral lubricant and an aliphatic nitrile having at least six carbon atoms.
2. As a new composition of matter, a mixture of a mineral lubricant and a mixture of aliphatic nitriles having at least six carbon atoms.
3. As a new composition of matter, a mixture of a mineral lubricating oil, stearo nitrile, and 45 palmito nitrile.
4. As a new composition of matter, a mixture of a mineral lubricating oil and cracked nitriles.
5. A penetrating oil including a mixture of aliphatic nitriles having at least six carbon atoms, 50
6. A penetrating oil including a mixture of stearo- and palmitonitrile.

ANDERSON W. RALSTON.

WILLIAM O. POOL.

JAMES HARWOOD.